

H. L. DOHERTY.

## METHOD OF CARBONIZING COAL.

APPLICATION FILED MAR. 21, 1913. RENEWED MAR. 11, 1916.

1,197,804.

Patented Sept. 12, 1916.

4 SHEETS—SHEET 1.

FIG. I



Witnesses: Charles Schabernack  
Chas. S. Reed

Henry L. Doherty Inventor  
By his Attorney Frank S. Young

1,197,804.

H. L. DOHERTY,  
METHOD OF CARBONIZING COAL,  
APPLICATION FILED MAR. 21, 1913. RENEWED MAR. 11, 1916.

Patented Sept. 12, 1916.

4 SHEETS—SHEET 2.

**FIG.2**



**FIG.3**



Witnessed: Charles Schabermack  
Chas. S. Reed

Chas. S. Reed

15-  
Henry L. Doherty Inventor  
By his Attorney Frank S. Young

1,197,804.

H. L. DOHERTY.

METHOD OF CARBONIZING COAL.

APPLICATION FILED MAR. 21, 1913. RENEWED MAR. 11, 1916.

Patented Sept. 12, 1916.

4 SHEETS—SHEET 3.



Witnesses: *Charles L. Abemethy*  
*Chas. L. Reed*

Henry L. Doherty Inventor  
By his Attorney, *Frank S. Young*.

1,197,804.

H. L. DOHERTY.  
METHOD OF CARBONIZING COAL.  
APPLICATION FILED MAR. 21, 1913. RENEWED MAR. 11, 1916.

Patented Sept. 12, 1916.

4 SHEETS—SHEET 4.

Fig. 5



Witnesses: Charles Schabermak  
Chas. S. Reed

Miss S. Reed

Henry L. Doherty Inventor

By his Attorney Frank S. Young.

# UNITED STATES PATENT OFFICE.

HENRY L. DOHERTY, OF NEW YORK, N. Y.

## METHOD OF CARBONIZING COAL.

1,197,804.

Specification of Letters Patent. Patented Sept. 12, 1916.

Application filed March 21, 1913. Serial No. 755,955. Renewed March 11, 1916. Serial No. 83,676.

To all whom it may concern:

Be it known that I, HENRY L. DOHERTY, a citizen of the United States, and a resident of New York city, in the county of New York and State of New York, have invented certain new and useful Improvements in Methods of Carbonizing Coal, of which the following is a specification.

This invention relates to methods of carbonizing coal and similar materials, and, in particular, to a method of continuous carbonization in shaft furnaces.

The objects of my invention are to supply to the art a continuous method of carbonizing fuel that will enable the carbonization to be carried out wholly, or in great part, by the heat developed by the carbonizing reactions themselves, effect the automatic gasification in the carbonizing apparatus of practically all of the heavier tar products, so that the gas will be taken off of the carbonizer practically free from all heavy pitch-forming constituents, and lamp black, and will permit of the withdrawal of the gas and coke from the carbonizer practically cold.

To this end, my invention, briefly stated, comprises the carrying out of the carbonization in a comparatively high shaft having a coal preheating and gas cooling section, a carbonizing section proper, a heat generating section, and a cooling section for the carbonized fuel, by circulating through the charge a suitable heat-carrying medium, the said heat-carrying medium being first passed in contact with the hot carbonized fuel in the lower part of the shaft, thence in contact with superheated coke or other carbonized fuel in a mid portion of the shaft, thence in contact with the material to be carbonized in the upper part of the shaft, whereby the said material is subjected to gradual heating to the temperature of carbonization while the circulating medium and the gas generated is cooled to be again introduced, in part, into the bottom of the shaft for the completion of another cycle. The superheating of the coke or carbonized material is performed by maintaining, either intermittently or continuously, a cross-draft of superheated air at the superheating section to heat the material to incandescence with the production of pro-

ducer gas which is burned to heat the air for the cross-draft. 55

I am aware that it has been proposed before to carry out the carbonization of coal in shaft furnaces by circulating gaseous fluids, but all of these have suffered from the defect that the extraneous heat which it is necessary to supply to the circulating medium owing to various losses, had to be supplied by transmission of heat to the gaseous fluid by conduction from exteriorly-heated walls. 65

One inventor proposes to return a portion of the gas drawn off of the top of the carbonizer to the base of the apparatus and pass the same upward through the hot carbonized coal to cool the same and to heat the returned gas. The heated gas then passes in contact with the coal in the upper portion of the shaft giving up heat to the same and effecting its carbonization. The heat losses are supplied by stopping the gas making operation during the drawing of the carbonized material and temporarily operating the carbonizing shaft as a gas producer by introducing air at the bottom and permitting it to ascend through the hot coke or other carbonized material. The result is the generation of producer gas which is burned in an annular jacket surrounding the carbonizing shaft proper, the heat so generated passing through the wall into the coal undergoing carbonization. The inventor also describes a modification of the above method in which he blasts a separate fuel bed to incandescence and carries the heat of the same into the carbonizing shaft by passing the cold returned gas through the said separate fuel bed and thence into the coal undergoing carbonization, instead of through the carbonized material. 80 85 90 95

Another method known to the art, performs the carbonization of the coal by heating a portion of the gas made in an exteriorly fired furnace and then passing it downward through the partially preheated coal to be carbonized. In this case the preheating is also performed by external heating of the shaft walls, while the cooling of the carbonized material is performed, wholly, by external cooling of the walls of the lower portion of the shaft. This method is still more objectionable than the 100 105

one previously mentioned in that it depends to a still greater extent upon external heating or cooling of the charge by conduction of heat, either to or from the same, through the shaft walls.

By my invention, on the other hand, I do away, entirely, with the necessity for the transmission of heat to or from the charge in the shaft through the shaft walls. All heating and cooling is done by directly contacting with the material a suitable fluid at a suitable temperature. The extreme distance to which the heat must be transmitted by conduction depends simply upon the size of the fragments of the charge and is measured by the shortest distance from the center of the largest fragment to the surface of the same. The heat required to institute the carbonizing action and to supply any necessary extraneous heat to the same is communicated to the carbonized material in the shaft itself by blasting the same with highly superheated air to form producer gas, which is burned to perform the superheating of the air.

The blasting of the coke or other carbonized material leaves it in a highly incandescent state. The circulating gaseous fluid, which has been used to quench the carbonized material in the lower part of the shaft and has thus itself been heated nearly or quite to the proper carbonizing temperature, is next passed in contact with the incandescent coke, to become superheated to the proper degree, and hence passes in contact with the material undergoing carbonization. By my invention there is, thus, no interference with the cooling of the coke during the period of extraneous heating of the material undergoing carbonization. The coke, which is subjected to the superheating, is that portion of the charge in the shaft which has just been carbonized and which is still at the maximum carbonizing temperature. There is no interference with the regular operation of the carbonizer and the operation of storing up heat in the coke to be transferred to the carbonizing charge may be carried out continuously without interfering with the carbonizing operation. Besides the ones enumerated, my invention comprises other features of increased utility which will be made plain below.

In the accompanying drawings I have shown an apparatus embodiment of my invention adapted to advantageously carry out the process features of the same.

Figure 1 is a vertical diametrical section through the shaft and its appurtenant regenerators on the line 1--1 of Fig. 2. Fig. 2 is a horizontal section through the same at the level 2--2 of Fig. 1. Fig. 3 is a plan of the apparatus with the operating floor removed. Fig. 4 is a partial front elevation of the same from the position indicated by

the line 4--4 of Fig. 3. Fig. 5 is a vertical section similar in position to Fig. 1 through a modified form of apparatus in which the superheating of the coke may be carried out continuously without interrupting the normal carbonizing operation.

In the drawings 1 indicates the carbonizing furnace or shaft, as a whole; 2 designates the fuel preheating section; 3 the carbonizing section proper; 4 the coke superheating section; and 5 designates the coke cooling section of the shaft.

It is to be understood that there is no sharp line of demarcation between the several sections of the shaft, but that the several regions, designated for convenience of reference by the several numerals mentioned, blend one into the other. The limits of the regions in which the several operations enumerated take place is largely a matter of the temperature existing at the different levels. The upper border of the coke superheating section (numbered 4) is more or less sharply defined by the level of the upper ports 28 in the apparatus of Fig. 1; but this is the only approximately fixed boundary plane separating the several sections. 6 and 6' are the regenerators.

7 is a blower for supplying air for blasting the coke during the superheating of the same, 8 is the discharge conduit of the blower 7, having branches 9 and 9' conducting air to the lower parts of regenerators 6 and 6', respectively. A by-pass 10, having a valve 32, serves to conduct a portion of the heated air from the upper part of one regenerator to the upper part of the other. Valves 12 and 12' on 9 and 9', respectively, serve to divert the flow of air from one conduit to the other, according to the direction of the "blow" through the carbonizer. These valves are usually arranged to be operated from the operating floor by means of operating gears 13 and 13', respectively, acting through elongated valve stems 14 and 14', respectively, which latter have on their upper ends racks which engage, respectively, with gears 13 and 13'. 15 is another blower, preferably of the positive type, which serves to circulate the gas or other heat-carrying medium through the charge in the shaft.

16 and 16' are condensers or scrubbers—16 for the portion of the circulating gas which is returned to the carbonizer and the other, 16', for the treatment of the gas going to the usual purifiers (not shown). In 16 the returned gas is, preferably, scrubbed with a portion of the tar oils (or some equivalent liquid which will absorb the illuminants from the gas). The gas returns to the carbonizer, therefore, comparatively free from those hydrocarbons which would be dissociated by repassing through the hot coke.

22 is the gas off-take leading from the

upper part of shaft 1, to the condenser-scrubbers 16 and 16', through the connections 38 and 39, respectively.

17 is the conduit which conducts the surplus gas from the condenser 16' to a relief holder, or directly to the scrubbers and purifying train, as may be desired.

The regenerators 6 and 6' each contain a checkerwork or some similar structure of refractory material.

The opposite walls, 18 and 18' of the shaft, in the superheating region 4, are, as shown, perforated with numerous ports (28 and 28', respectively,) communicating directly with the upper portion of the regenerator chambers. This arrangement permits of the cross-blasting of the charge in the shaft in either direction. The shaft, itself, may be advantageously constructed, as shown, of a rectangular cross-section, with rounded corners. If for any reason preferred, however, the cross-section may be circular or elliptical. A door, 19, permits of the charging of the raw coal, while a discharging device, 20, permits of the drawing of the relatively cold coke from the bottom of the shaft without interfering with the gas making operation.

The method of operation is as follows: In starting operations, the shaft is, preferably, filled to near the bottom of the superheating section 4 with coke. Kindling is charged upon this and ignited. During this stage, the charging door 19 may advantageously be left open and likewise the discharging door 21, near the bottom of the shaft. The combustion is thus sustained by the natural draft of the shaft. Coal or coke is now gradually charged upon the ignited kindling until a mass of ignited fuel has

been built up to above the section 4. The coal which is to be carbonized is now charged into the shaft up to the level at which it is intended to carry it, either alone or mixed with coke. The charging door 19 and the discharging door 21 at the bottom of the shaft are both closed and the blower 15 set in operation. The gas generated from the raw coal passes off from the upper part of the shaft through the conduit 22 and thence

divides, one stream going to the condenser 16 and the other to the condenser 16'. The distribution of the gas between 16 and 16' may be regulated by the valves 24 and 27. The blower 15 draws off the gas from 16 through the conduit 23 and forces it through the conduit 25 into the lower part of the cooler 5 of the shaft 1. This gas passes up through the relatively cold coke in the lower part of the shaft, thence through the hot coke in 4.

From 4, the heated gas passes into the coal in the upper portions 3 and 2 of shaft 1. As the hot gas ascends, it gradually gives up its heat to the coal, raising the lower portion of the mass in 3 to the temperature of carbonization and subjects the mass above

to gradual heating. When the temperature of the hot coke in 4 has fallen below that necessary to communicate the required heat to the gas, the valves 26 and 27 are closed, valves 12 and 12' adjusted, for example, to admit air into the lower part of 6. This is effected by closing valve 12' and opening valve 12. Blower 7 is started by setting its motor 7' in operation and air now passes up through the checker 37 in regenerator 6' (which at the start is necessarily cold) and thence through the ports or nostrils 28 into the ignited coke in 4. The stack valve 29' on the connection 30' from the lower part of 6', being open, a draft is established across the section 4 through the hot coke, through the nostrils 28' into and down through the checkerwork 37' in regenerator 6'. The nostrils 28' may be located directly across the shaft from the nostrils 28, or may be located at a level either above or below the nostrils 28. With shafts of large cross-section, they are, preferably, located opposite the nostrils 28. With shafts of small cross-section, the nostrils 28' are usually located at either a higher or lower level than the nostrils 28, in order to secure the proper thickness of fuel for the draft current to traverse. In its passage across the fuel bed, the oxygen of the draft promotes a rapid combustion in the prism of coke or other carbonized material, heating the same to incandescence. The combustion instituted by the oxygen of the air is usually, principally, to-carbon monoxide, forming usually, a relatively poor producer gas. This passes through the nostrils 28' (when the flow in superheating section 4 is in the direction from left to right) as stated, and in the upper part of regenerator 6' meets the air discharged into 6' from the by-pass 10.

The distribution of the air from regenerator 6, between section 4 of the shaft and regenerator 6' is effected by the setting of the valve 32, which may be an ordinary hand-operated valve. This valve should be so set that the volume of air flowing through 10' may be just sufficient to burn the combustible constituents generated by the blasting of the fuel column in 4 by the air passing through nostrils 28. The actual distribution of the air between the section 4 of shaft 1 and regenerator 6' will depend, principally, upon the pressure at which the air is supplied. When the blast pressure used is comparatively high, the proportion of the oxygen of the blast which is burned to  $CO_2$  in 4 (or rather which leaves 4 as  $CO_2$ ) is relatively high, while the proportion of  $CO$  in the effluent gas is relatively low. This condition, therefore, would permit of much the larger portion of the air being sent through the coke in section 4, since, in this case, a part of the combustion which would otherwise occur in regenerator 6' is

transferred to superheating section 4. This is a decided advantage, inasmuch as much less air is required to produce a given temperature increment in the carbonized material in 4, and the duration of the blasting period of "blow" is greatly shortened both on account of the less volume of air required and the greater pressure (and hence velocity), under which it is supplied. With 5 a low blast pressure, on the other hand, the proportion of CO in the effluent gases is increased and a larger proportion of the total air used is required in regenerator 6'. Inasmuch, however, as the CO produced in 4 is 10 utilized to heat the air for the subsequent blow in the reverse direction, the actual quantity of air required to be passed through the superheating chamber 4 is not increased in the ratio that would otherwise be indicated by the lower ratio of CO<sub>2</sub> to CO. Owing to the relatively low percentage of 15 heat utilization in the regenerators as compared with that in the superheating chamber, however, it is usually desirable to use 20 the blast under comparatively high pressure (20 to 30 inches of water). The distribution of air between 4 and 6' having been properly adjusted by the manipulation of the valve 32, the combustible 25 constituents of the gas entering regenerator 6' will be completely burned in the checker of the regenerator, the combustion gases giving up the greater part of their heat to the same, if the capacity of the regenerators has been properly adjusted to the 30 duty required of them. The comparatively cool combustion gases discharge from the lower part of the regenerator through the conduit 30' and pass to the chimney 31. 35 When the proper temperature has been attained in the carbonizing chamber, the switch controlling motor 7' is opened, stopping the blower 7, and valve 12 shut. Valves 26 and 27 are again opened and motor 15' 40 started. Gas again passes up through cooler 5, superheating section 4, where it is more or less superheated, and thence through the coal (or other material) undergoing carbonization, giving up heat to the same and 45 supporting its carbonization as before described. Since the relative heat capacity of the stream of coal is somewhat greater under normal conditions than the heat capacity of the oppositely flowing stream of gas, the latter will leave the upper part of the shaft comparatively cool. Owing to the "lag" in the conduction of heat, however, the gas usually leaves the shaft 1 at a temperature around 150 to 250 degrees F. At 50 this temperature, of course, nearly all of the vapors produced in the carbonization are condensed, and scrubbed out of the gas by the coal in the preheating chamber 2. The gas thus leaves the carbonizer in a fair 55 pure condition carrying, for the most part,

only such impurities as are permanent gases (so called) together with a small amount of hydrocarbons of low boiling point and water vapor. These latter are condensed in the condensers 16 and 16', leaving the gas 70 clean and in admirable condition to undergo the ordinary purification treatment.

The condensation of tarry matter in the coal in preheating chamber 2, if permitted to proceed uninterrupted, would eventually 75 impede the flow of the gases and clog the operation of the carbonizer. To correct this tendency I, at intervals, change the direction of the run, passing the circulating gaseous stream downward through the material undergoing carbonization. This is effected by closing valves 26 and 27 on connections 22 and 25 and opening valves 33 and 34 on connections 35 and 36, respectively. The blower 15 now forces the gas, 80 which it draws from the condenser and scrubber 16, through conduits 25 and 36 to the upper part of fuel-preheating chamber 2 of shaft 1, thence down through the shaft and through conduit 35 to condensers 16 85 and 16'. In passing down through the interstices of the charge, the gas carries downward the accumulated tarry matter into the hottest region of the shaft in the superheating section 4. In contact with the hot 90 coke, the tar-forming compounds are broken up to form permanent gases, difficultly-condensable hydrocarbons and free carbon. The returned gas, together with the new gas generated, passes down through 95 the shaft in contact with the previously cooled coke in the cooler 5, giving up most of its sensible heat to the same, and thence passes to the condensers, as before described. Since the apparatus is so designed and operated that in normal working there will 100 always be a considerable body of cold coke in chamber 5, and since the duration of the down blow is comparatively brief, the relatively high temperature region in the shaft 105 will not be carried downward to an extent that will interfere with the working upon returning to the normal "up-runs". This method of securing the gasification of matter condensed in the upper part of the fuel 110 column, by reversing the normal direction of the run, I do not claim specifically herein, that forming a specific feature of the invention disclosed in my application Ser. No. 660,450, referred to above. This element is 115 only claimed herein in connection with other elements of the specific process disclosed.

When the temperature in the superheating chamber 4 has again fallen below that required for proper carbonization, the blower 15 is again shut down, the valves 12 on the gas connections on the shaft 1 closed, blower 7 started, valve 12 opened and valve 32 is adjusted to give the proper distribution of the air between 6' and 4. Air now 120 125 130

flows through 9' to the lower part of regenerator 6', passes up through the previously heated checkerwork in the same, thence through the nostrils 28' into the 5 superheating chamber 4. Passing through the coke in 4, combustion is again instituted with the formation of more or less combustible gas, and the reheating of the coke. The effluent gas passes through the nostrils 10 28 into the regenerator 6. Then it mingles with the air flowing to 6 through the bypass 10 and burns. The combustion gases pass down through the checker 37 in 6 giving up most of their heat to the same, 15 thence flow through conduit 30 (valve 29 being open) to the chimney 31. If desired, a boiler for generating steam, or other heat utilizing apparatus may be interposed between the stack and the regenerators. 20 The relative duration of the "runs" and "blows" will vary with the character of the coal used, the cross dimension of the stack and various other considerations. The larger the cross section of the stack the less 25 is the radiating surface compared with the quantity of material under treatment and consequently the less is the percentage heat loss. With a comparatively large cross section of the stack, with some coals, the carbonizer having once been put in normal 30 operating condition, the carbonization may be sustained indefinitely without having recourse to blasting to recoup heat losses. With other fuels, more or less frequent 35 blasting may be required to maintain the temperature at the proper point for carbonization. Working with apparatus of comparatively small cross section and with a gas coal of only average quality, I have 40 found that four minutes blasting to thirty minutes of "run" will amply suffice to maintain the temperature of the carbonizer. 45 The movement of the charge through the carbonizer may be either continuous or intermittent. As fast as the relatively cold coke is removed at the bottom of the shaft, coal is, of course, charged in at the top, so that the charge in the shaft is always maintained at substantially the same level. 50 With most coals it is advantageous to feed with the coal a certain proportion of coke, after the method disclosed by me in applications. Ser. Nos. 660,450; 660,451, 660,453, and 670,338. The object of admixing preformed coke with the coal charged 55 is to prevent the formation of large coke aggregates which would offer obstruction to the passage of the blast, forcing the draft current to the walls and thus interfere with 60 the uniform distribution of the draft throughout the body of the charge. This latter requirement is of special importance in the practice of my invention in that I depend upon the direct contact between the 65 circulating heat-carrying medium and the

fragments of the charge for the transfer of heat from one portion of the charge to the other.

When deemed desirable, steam may be used in admixture with the returned gas, 70 or even used alone as the heat-carrying medium. When the carbonization is carried on at a comparatively high temperature, above 1800 degrees F., the presence of steam in the gas returned, of course, involves a proportionate combustion of coke to form water gas. When carrying on the carbonization at a relatively low temperature, say 1000 degrees to 1200 F., steam alone may be used as the heat-carrying medium without 75 the formation of any great amount of water gas. In this case, it is, of course, necessary to so operate the apparatus that the coke and gas will both be withdrawn at temperature above 212° F. The steam 80 withdrawn may be separated from the gas by condensation. It has been determined by experiment that coal may be practically completely carbonized at a temperature as low as 800 degrees F., when the time of 85 treatment is sufficiently prolonged. When carbonized at this temperature, while the make of gas is low, the candle power per ton of coal and the value of the condensation products are high. With apparatus in common use, however, it is difficult to maintain 90 the necessary uniform low temperature throughout the charge. Therefore, carbonization at low temperatures has been but little used. My invention, however, is peculiarly well suited to carrying out the low 95 temperature distillation of coal. In cases where the coal is sufficiently exothermic in its carbonization, and where the apparatus is properly designed, after the carbonization has once been properly established, it 100 may be maintained indefinitely at temperatures as low as 900 degrees to 1000 degrees F.

By means of the apparatus embodiment 110 of my invention shown in Fig. 5, the blasting of the coke may be carried out without any interruption of the make of gas. In this, the chamber in which the coke is blasted is not traversed by the circulating gaseous 115 heat-carrying medium.

The method of operation is as follows: The coal is, as before, preheated in a pre-heating chamber 2, carbonized in a lower portion 3 of the shaft 1, blasted in a mid-section 4, and quenched and cooled in cooler 5 in the lower portion of the shaft. The circulating gas, however, is withdrawn from the shaft traversing before the superheating chamber 4, through the flue 40, by the fans 120 41, and reintroduced again into the shaft through the conduit 42 above the chamber 4. In this type of apparatus I, preferably, although not necessarily, use a regenerator of 125 the double surface type, commonly called 130

recuperators in the art. In this type the air flows through the flues 43, of the recuperator 44, to the superheating chamber 4, through the coke occupying this chamber, burning more or less of the latter to form producer gas and to heat the coke. Under the induction exerted by the chimney 45, the producer gas flows into and through the conduit 46, thence through the flues 47 of the recuperator 44. Air is admitted to the flues 47 through the dampers 48, burning the combustible constituents of the producer gas. The heat generated is to a large extent transmitted through the flue walls to the inflowing air passing through the flues 43. The air thus reaches the superheating chamber 4 at a high temperature and but little combustion is necessary to impart a suitable temperature to the coke. The spent combustion gases from the flues 47 flow to the chimney 45, which supplies the inductive effect necessary to draw in the air through the dampers 48. As coke is withdrawn at the bottom of the shaft, the heated coke in 4 descends into the upper part of the cooler 5 and is thus brought into contact with the ascending stream of circulating gas.

The operation of this modification of my invention is, in other respects than the ones just described, essentially the same as in the case of the first form of apparatus.

I claim:

1. The process of carbonizing fuel and producing gas which comprises advancing a body of material containing the fuel to be carbonized downwardly through a relatively long conduit, maintaining a carbonizing temperature at a mid-region in said conduit by burning a portion of the carbonized fuel in said mid-region by passing laterally therethrough a combustion supporting draft current, withdrawing cool distillation gas from the upper part of said conduit, diverting a portion of the distillation gas, passing the said diverted gas upwardly through the hot carbonized fuel advancing from said mid-region, thence in contact with the hot carbonizing fuel in said mid-region, thence through the material in the upper portion of said conduit in admixture with the distillation gases from said carbonizing region.

2. The process of carbonizing fuel and producing gas which comprises advancing a body of material containing the fuel to be carbonized downwardly through a relatively long conduit, maintaining a carbonizing temperature at a mid-region in said conduit by burning a portion of the carbonized fuel in said region by passing laterally therethrough a combustion supporting draft current, cooling the carbonized material that has advanced beyond said mid-region by passing upwardly therethrough a current of initially cool gaseous fluid, passing said

gaseous fluid through the hot carbonized material in said mid-region thence through the material above said mid-region, whereby the lower portion of said material above said region is subjected to a carbonizing temperature and the material in the upper portion of said material above said region is subjected to preheating, while the said gaseous fluid and the distillation gases from the carbonized material are cooled, and withdrawing the cooled gases from the upper part of said conduit.

3. The process of carbonizing fuel and producing gas which comprises advancing a body of material containing the fuel to be carbonized downwardly through a relatively long conduit, maintaining a carbonizing temperature at a mid-region in said conduit by burning a portion of the carbonized fuel in said region by intermittently passing laterally therethrough a combustion supporting draft current, cooling the carbonized material that has advanced beyond said mid-region by passing upwardly therethrough a current of initially cool gaseous fluid, passing said gaseous fluid through the hot carbonized material in said mid-region, thence through the portion of the material above said mid-region whereby the lower part of the said portion of material is subjected to carbonization while the upper part of said portion of the material is subjected to preheating, while the said gaseous fluid and the distillation gases produced in the carbonization of said material are cooled, and withdrawing the cooled gases from the upper part of said conduit.

4. The process of carbonizing fuel and producing distillation gases which comprises advancing a body of material containing the fuel downwardly through a relatively long conduit, maintaining a carbonizing temperature at a mid-region in said conduit by passing laterally through carbonized material in said mid-region a stream of preheated air, cooling the carbonized material that has advanced beyond said mid-region by passing upwardly therethrough a current of initially cool gaseous fluid, passing said gaseous fluid through the hot carbonized material in said mid-region, thence through the material above said mid-region, whereby the lower portion of the said material above said mid-region is subjected to a carbonizing temperature and the upper portion of said material is subjected to preheating, while the said gaseous fluid and the distillation gases from the carbonized material are cooled, and withdrawing the cooled gases from the upper part of said conduit.

5. The process of carbonizing fuel and producing distillation gases which comprises advancing a body of material containing the fuel downwardly through a relatively long conduit, maintaining a carbonizing temper-

- ature at a mid-region in said conduit by intermittently passing laterally through carbonized material in said mid-region a stream of preheated air, to produce combustible gas 5 and to heat said carbonized material, withdrawing the so-produced combustible gas and burning the same to heat air, passing upwardly through the carbonized material that has advanced beyond said mid-region 10 a current of initially cool gaseous fluid, whereby the said carbonized material is cooled and the said gaseous fluid heated, passing the so-heated gaseous fluid through the heated carbonized material in said mid-region to further heat said fluid, thence 15 through the material in the part of said conduit above said mid-region, whereby the lower portion of said material is subjected to carbonization and the upper portion of 20 said material is preheated, while the said gaseous fluid and the distillation gases from the carbonization of said fuel are cooled, and withdrawing the cooled gases from the upper part of said conduit.
6. The process of carbonizing fuel and producing distillation gases which comprises advancing a body of material containing the fuel downwardly through a relatively long conduit, maintaining a carbonizing temperature at a mid-region of 25 said conduit by intermittently passing laterally through carbonized material in said mid-region, first in one direction and then in the reverse direction, a current of pre-heated air to produce combustible gas and to heat said carbonized fuel, withdrawing the so-produced combustible gas from said conduit and burning the same to heat air for the reverse blast, passing upwardly 30 through the carbonized material below said mid-region a current of initially cool gaseous fluid, whereby the said carbonized material is cooled and the said gaseous fluid heated, passing the so-heated gaseous fluid 35 through the heated carbonized material in said mid-region to further heat said gaseous fluid, thence through the material in the part of said conduit above said mid-region whereby the lower portion of said 40 material is subjected to carbonization and the upper portion of said material is heated, while the said gaseous fluid and the distillation gases from the carbonization of said fuel are cooled, and withdrawing the cooled 45 gases from the upper part of said conduit.
7. The process of carbonizing fuel and producing distillation gases which comprises advancing a body of material containing the fuel downwardly, through a relatively long conduit, maintaining a carbonizing temperature at a mid-region of 50 said conduit by intermittently blowing laterally through carbonized material in said mid-region, first in one direction and then in the reverse direction a current of pre- 55 heated air to produce combustible gas and to heat said carbonized fuel, withdrawing the combustible gas formed during the blow in one direction and burning said gas to heat air to be used in the blow in the reverse direction, withdrawing distillation gas from the upper part of said conduit, diverting a portion of the distillation gas withdrawn, introducing said diverted gas into the lower part of said conduit and passing the said gas upwardly in contact with the carbonized material discharged from the said mid-region to preheat said gas and to cool said carbonized material, passing the preheated gas in contact with the heated carbonized material in said mid-region to further heat said gas, and passing said gas through the material above said mid-region to carbonize the lower portion of said material and to preheat the upper portion of said material. 60
8. The process of carbonizing fuel and producing distillation gases which comprises advancing a body initially composed of fresh fuel and carbonized material downwardly through a relatively long conduit, maintaining a carbonizing temperature at a mid-region of said conduit by intermittently blowing laterally through carbonized material in said mid-region, first in one direction and then in the reverse direction a current of preheated air to produce combustible gas and to heat said carbonized fuel, withdrawing the combustible gas 65 formed during the blow in one direction and burning said gas to heat air to be used in the blow in the reverse direction, withdrawing distillation gas from the upper part of said conduit, diverting a portion of the distillation gas withdrawn, introducing said diverted gas into the lower part of said conduit and passing the said gas upwardly in contact with the carbonized material discharged from the said mid-region to preheat said gas and to cool said carbonized material, passing the preheated gas in contact with the heated carbonized material in said mid-region to further heat said gas, passing said gas through that portion of said fuel mixture above said mid-region to carbonize the fuel in the lower part of said 70 portion and to preheat the fuel mixture in the upper part of said fuel mixture, withdrawing cool carbonized material from the bottom of said conduit and returning part of said carbonized material in admixture with fresh fuel to the upper part of said conduit.
9. The process of carbonizing fuel and producing distillation gases which comprises advancing a body of material initially composed of fresh fuel and carbonized material in admixture downwardly through a relatively long conduit, maintaining a carbonizing temperature at a mid-region in said conduit by burning a portion of the car- 75 80 85 90 95 100 105 110 115 120 125 130

- bonized fuel in said mid-region by passing laterally therethrough a combustion supporting draft current, withdrawing cool distillation gas from the upper part of said conduit, diverting a portion of the distillation gas, passing the said diverted gas upwardly through the hot carbonized fuel advancing beyond said mid-region, thence in contact with the hot carbonizing fuel in said mid-region, thence through the material in the upper portion of said conduit in admixture with the distillation gases from said carbonizing region, withdrawing cool carbonized fuel from the bottom of said conduit, and admixing part of said carbonized material with fresh fuel for repassage through said conduit.
10. The process of carbonizing fuel and producing gas which comprises advancing a body initially composed of fresh fuel and carbonized fuel downwardly through a relatively long conduit, maintaining a carbonizing temperature at a mid-region in said conduit by burning a portion of the carbonized fuel in said region by passing laterally therethrough a combustion supporting draft current, cooling the carbonized material that has advanced beyond said mid-region by passing upwardly therethrough a current of initially cool gaseous fluid, passing said gaseous fluid through the hot carbonized material in said mid-region, thence through the portion of the material above said mid-region, whereby the lower part of said portion of said material is subjected to a carbonizing temperature and the material in the upper part of said portion of said material is subjected to preheating, while the said gaseous fluid introduced and the distillation gases from the carbonized material are cooled, withdrawing the cooled gases from said conduit, withdrawing cool carbonized material from said conduit, admixing a portion of the carbonized material withdrawn with fresh fuel and feeding said mixture on to the top of said fuel body.
11. The process of carbonizing fuel and producing gas which comprises advancing a body of material containing the fuel to be carbonized downwardly through a relatively long conduit, maintaining a carbonizing temperature at a mid-region in said conduit by burning a portion of the carbonized fuel in said mid-region by passing laterally therethrough a combustion supporting draft-current, normally withdrawing cool distillation gas from the upper part of said conduit, diverting a portion of the distillation gas, passing the said diverted gas upwardly through the hot carbonized fuel advancing from said mid-region, thence in contact with the hot carbonizing fuel in said mid-region, thence through the material in the upper portion of said conduit in admixture with the distillation gases from said carbonizing region, and periodically reversing the direction of flow of said diverted distillation gases, said diverted gases passing during reversal first in contact with the raw fuel, thence into and through the hot carbonized fuel in said mid-region, whereby tarry matter condensed in said raw fuel is carried down into contact with said hot carbonized fuel and gasified, withdrawing the gases formed from a locality below said mid-region, diverting a portion of said diverted gases and returning said diverted gases to the upper part of said fuel body.
12. The process of carbonizing fuel and producing gas which comprises advancing a body of material containing the fuel to be carbonized downwardly through a relatively long conduit, maintaining a carbonizing temperature at a mid-region in said conduit by burning a portion of the carbonized fuel in said region by passing laterally therethrough a combustion supporting draft current, normally cooling the carbonized material that has advanced beyond said mid-region by passing upwardly therethrough a current of initially cool gaseous fluid, thence passing said gaseous fluid through the hot carbonized material in said mid-region, thence through the material above said mid-region, whereby the lower portion of said material is subjected to a carbonizing temperature, the upper portion of said material to preheating and tarry constituents condensed out of said gaseous fluid, periodically reversing the direction of flow of said gaseous fluid by passing the same first through the upper portion of said fuel body above said mid-region, thence downwardly through the hot carbonized fuel in said mid-region, whereby said condensed tarry constituents are gasified, withdrawing cool distillation gas from the upper portion of said fuel body during normal flow of said gaseous fluid and from the lower part of said fuel body during reversal.
13. The process of carbonizing fuel and producing gas which comprises advancing a body of material containing the fuel to be carbonized downwardly through a relatively long conduit, maintaining a carbonizing temperature at a mid-region in said conduit by burning a portion of the carbonized fuel in said region by intermittently passing laterally therethrough a combustion supporting draft current, normally cooling the carbonized material that has advanced beyond said mid-region by passing upwardly therethrough a current of initially cool gaseous fluid, thence passing said gaseous fluid through the hot carbonized material in said mid-region, thence through the portion of the material above said mid-region, whereby the lower part of said portion of the material is subjected to carbonization, the upper part of said portion of the material

to preheating, while the said gaseous fluid and the distillation gases produced in the carbonization of said material are cooled and tarry liquid condensed therefrom, periodically reversing the direction of flow of said gaseous fluid by passing the same first through the portion of said fuel body above said mid-region, thence through the hot carbonized fuel in said mid-region, whereby said condensed tarry liquid is gasified, normally withdrawing cool distillation gases from the upper portion of said fuel body during normal flow of said gaseous fluid and from the lower portion of said fuel body during reversal.

11. The process of carbonizing fuel and producing distillation gases which comprises advancing a body of material initially composed of fresh fuel and carbonized fuel in admixture downwardly through a relatively long conduit, maintaining a carbonizing temperature at a mid-region in said conduit by burning a portion of the carbonized fuel in said mid-region by passing laterally therethrough a combustion supporting draft current, normally withdrawing cool distillation gas from the upper part of said conduit, diverting a portion of said distillation gas, normally passing said diverted gas upwardly through the initially hot carbonized fuel advancing beyond said mid-region, thence in contact

with the hot carbonized fuel in said mid-region, thence through the portion of said body of material above said mid-region to 35 carbonize fresh fuel, thence in admixture with the distillation gases from the carbonized fresh fuel through the upper portion of said body of material to preheat said material, to cool said gases and to condense 40 tarry liquid from said gases, periodically reversing the flow of said distillation gases, withdrawing cool distillation gases from the lower part of said fuel body, diverting a portion of said distillation gases, passing 45 said diverted portion of said distillation gases downwardly through the mixture of fresh and carbonized fuel in the upper portion of said fuel body, thence through the hot carbonized fuel in said mid-region, whereby said condensed tarry liquid is gasified, withdrawing cool carbonized fuel from the bottom of said conduit, admixing a portion of said carbonized material with fresh fuel and introducing the said mixture into 55 the upper part of said conduit.

Signed at New York city, in the county of New York and State of New York, this 17th day of Mar., A. D. 1913.

HENRY L. DOHERTY.

Witnesses:

WILLIAM C. DREYFUS,  
THOS. I. CARTER.